

## 1

3,016,298

ONE-COMPONENT DIAZOTYPE MATERIAL  
 Theodorus Petrus Wilhelmus Sanders, Venlo, and Hubertus Wilhelmus Henricus Maria Roncken, Roermond, Netherlands, assignors to Chemische Fabriek L. van der Grinten N.V., Venlo, Netherlands, a corporation of the Netherlands  
 No Drawing. Filed June 16, 1958, Ser. No. 742,025  
 Claims priority, application Netherlands June 17, 1957  
 13 Claims. (Cl. 96—75)

The invention relates to one-component diazotype material the light-sensitive layer of which contains a diazo compound and an organic acid.

As is known, in the so-called one-component diazotype process use is made of light-sensitive materials the light-sensitive layer of which contains one or more diazo compounds and one or more acids or acid-reacting salts, and of developing liquids, generally consisting of aqueous solutions of one or more coupling components and means, such as alkalis, buffer salts or mixtures thereof, which neutralize the acid present in the light-sensitive layer and enable the formation of the azo-dyestuff. In the so-called semi-wet diazotype process development is effected by coating the surface of the imagewise exposed diazotype material evenly with a thin layer of developing liquid of, for example, 8 g. per m.<sup>2</sup>. This developing liquid must be able, in the short time in which a thin layer of it dries up on the surface of the diazotype material, to transform essentially all the diazo compound present on the diazotype material into azo-dyestuff of the desired colour, in other words to bring about a substantially complete development of the diazotype material.

In this connection the coupling activity of the diazo compounds and azo coupling components used is naturally of great importance. The conditions which are important for substantially complete development always have to be adapted to the coupling activity of the diazo compounds and azo coupling components used. In order to obtain substantially complete development, the acid content of the light-sensitive layer and accordingly its pH and/or its buffer capacity, and/or the percentage of alkalis and/or buffer salts of the developing liquid and accordingly the pH and/or the buffer capacity of that liquid, may be varied in proportion to the coupling activity of the diazo compounds used for the sensitization of the one-component diazotype material. In order to minimize or avoid deleterious effect on the keeping quality of the developed diazotype copy, on its mechanical strength, for example, its tearing-resistance, and on the fastness of the azo-dyestuff and of the background of the copy, for example, on exposure to light, and in order to maintain keeping quality, and freedom from crystallization, and to prevent etching activity of the developing liquid, it is endeavoured to keep the acid content of the light-sensitive layer and the percentage of alkalis or buffer salts of the developing liquid at a low value.

Developers reacting moderately alkaline are therefore preferred to those reacting strongly alkaline, and developers with a low percentage of buffer salts to those with a high percentage of buffer salts. A developing liquid reacting moderately alkaline has a pH between 8 and 11 and contains alkali salts, such as borates, carbonates, and phosphates. The coupling component it contains is generally phloroglucinol, a very actively coupling compound, which is able to couple at one, two or three places with the diazo compound and in proportion thereto forms dyestuffs of various shades.

In order to obtain certain neutral shades, use is also made of a mixture of phloroglucinol with other coupling components, for example, resorcinol.

With such developers reacting moderately alkaline substantially complete development is achieved by the semi-

## 2

wet development of one-component diazotype material which has been sensitized with diazo compounds having a great coupling activity, such as p-diazo di-phenylamine, p-diazo o-chloro N-monocyclohexylaniline, p-diazo N,N-di-n-butylaniline, p-diazo N,N-di-n-hexylaniline, p-diazo N-ethyl N-benzylaniline, p-diazo o-methyl N,N-diethyl-aniline, p-diazo o-chloro N,N-diethylaniline, and certain p-diazo o-alkoxy N,N-dialkylanilines, such as p-diazo o-ethoxy N,N-di-n-propylaniline and p-diazo o-methoxy N-ethyl N-benzylaniline.

Diazo compounds coupling even more actively than those just referred to are compounds such as 4-diazo 2,5-dialkoxy acylanilides, for example, 4-diazo 2,5-diethoxy benzylidene, 4-diazo 2,5-dialkoxy arylmercaptobenzene compounds and 4-diazo 2,5-dialkoxy diphenyl compounds. Less actively coupling diazo compounds are compounds such as p-diazo N,N-dimethylaniline, p-diazo N,N-diethylaniline, p-diazo m,methyl-N,N-dimethylaniline, and diazo-anhydrides such as 2-diazo-1-naphthol-5-sulphonic acid. On account of their small coupling activity these less actively coupling diazo compounds are not suited for the semi-wet development with the said developers reacting moderately alkaline. The coupling activity of the diazo compounds can be determined comparatively *in vitro* by measuring the time in which a given portion (for example, 10%) of the diazo compound to be examined will have coupled in a given molar concentration (for example, 0.1 millimolar) with the coupling component 1-phenyl 3-methyl pyrazolone-(5) in a given molar concentration (for example, 1.0 millimolar) in a buffer mixture of a given composition and a given pH at a given temperature.

Diazotype materials sensitized with the above-mentioned very actively coupling diazo compounds of the groups of 4-diazo 2,5-dialkoxy acylanilide, 4-diazo 2,5-dialkoxy-arylmercaptobenzene, 4-diazo 2,5-dialkoxydiphenyl, as far as their coupling activity is concerned are suited for semi-wet development with very weakly alkaline, neutral or even weakly acidic but strongly buffered developers.

With such developers containing phloroglucinol they are able to give fine black azo-dyestuffs. With the said developers reacting moderately alkaline, however, they yield azo-dyestuffs with less pure (or less neutral) shades, generally lighter-coloured, for example, brownish or purplish shades of colour, because during development the pH of the surface of the diazotype material, notwithstanding the moderately alkaline reaction of the developing liquid, is still too high in relation to the very great coupling activity of the diazo compounds. This is called "over-development."

Efforts have been made to manufacture with the said very actively coupling diazo compounds diazotype materials which are suited for semi-wet development with the said developers reacting moderately alkaline, and which in this process will not be over-developed, but give pure (or neutral) azo-dyestuff shades. For this purpose the light-sensitive layer of these diazotype materials has been given a high content of acid. Whilst the sensitizing liquids for the manufacture of diazotype materials with these diazo compounds usually contain only approximately 0.5-1% of their weight of the acids normally used in one-component diazotype layers, such as tartaric acid, citric acid, aluminum sulphate, alum, and the like, and the diazotype materials produced therewith are then suited for semi-wet development with weakly alkaline to weakly acidic buffered developers, they have to contain about 3 to 4% of these acids for the manufacture of diazotype materials which are suited for the semi-wet development with the above-mentioned developers reacting moderately alkaline.

Though the buffering capacity of the light-sensitive

layer of one-component diazotype materials which contain so large a quantity of such an acid is higher than that of the corresponding materials containing a small amount of acid, it is nevertheless insufficient for the practice of the semi-wet diazotype process with the said developers reacting moderately alkaline. In fact, the materials are very sensitive to development fluctuations when such developers containing polyvalent azo coupling components, such as phloroglucinol, are used. These fluctuations generally arise because the quantity of developer applied itself fluctuates, for example, owing to shocks or vibrations of the developing apparatus or when its speed is changed. Other causes may be a change in the concentration of the developers, for example, through a mistake in the preparation of the solution or owing to evaporation of the latter during use or slight irregularities in the light-sensitive layer owing to which it does not take up the developer quite uniformly. In current practice development fluctuations now occur to a greater extent since formerly a large excess of dilute developer was used whereas in the modern semi-wet diazotype process the quantity of developer applied per unit-surface, which developer is generally used in a more concentrated form, is kept small. The sensitivity of the light-sensitive layer to development fluctuations is shown by shifts in shades in the colours of the image, for example, by deviations from the desired neutral black. If, for example, a neutral black colour is obtained with a developer of the correct concentration containing phloroglucinol, a violet-black shade is obtained with a developer which contains only 80% of the usual quantity of water or has been evaporated to this value, whilst with a developer which is too dilute a green-black shade is obtained and often not all of the diazo compound is converted into azo-dyestuff.

Diazotype material, especially diazotype paper, which contains such large quantities of the said fairly strong acids, upon ageing also shows a considerable decrease of its mechanical strength, which appears, for example, from a reduced tearing-resistance.

In order to avoid the objectionable consequences of development fluctuations in the semi-wet development of diazo film layers, it has been proposed to sensitize diazo film layers with a p-diazo-dialkylaminobenzene compound each alkyl group of which contains at least 4 and at most 7 C-atoms, while both alkyl groups contain together 10, 11 or 12 C-atoms and at most one of the two alkyl groups carries a side-chain attached to the  $\alpha$ -C-atom. These diazo compounds couple actively and the diazo film layers sensitized with them are suited for the semi-wet development with the said developers reacting moderately alkaline. These diazo film layers contain very small quantities of the acids normally used in the diazotype process, such as tartaric acid, citric acid, and alum.

Besides tartaric acid and citric acid, other organic acids or their salts have also been applied in the light-sensitive layer of diazotype materials.

Thus, a process is known for deepening the shades of colour when one-component diazotype material which has been sensitized with p-amino-benzene diazo compounds is used. In this process an unsaturated organic compound with one or more carbon double bonds, for example, the sodium salt of maleic acid, itaconic acid or citraconic acid, is used in the light-sensitive layer or in the developer. This process has been applied, for example, with less actively coupling diazo compounds, such as p-diazo-N,N-diethylaniline. The said salts have a detrimental effect on the keeping quality of one-component diazotype material with actively coupling diazo compounds. Even upon application of free itaconic acid, the keeping quality of such material is very poor. Moreover, itaconic acid and citraconic acid are rather expensive.

It has further been proposed to manufacture light-sensitive layers with the aid of reaction products of diazo-

anhydrides with salts of organic aliphatic or aromatic acids, such as acetic acid, lactic acid, tartaric acid, citric acid, oxalic acid, succinic acid, benzoic acid, and benzene sulphonic acid. Such layers naturally contain only a small quantity of an acid combined with the diazo molecule. The coupling activity of diazo-anhydrides is very low, so that they are not suitable for application in one-component diazotype material for the semi-wet diazotype process with a developer reacting moderately alkaline.

According to the present invention a one-component diazotype material has a light-sensitive layer which contains a diazo compound coupling at least as actively as p-diazo diphenylamine, preferably a diazo compound that can readily couple with phloroglucinol in an acid medium and an aliphatic saturated dicarboxylic acid in which the carboxylic acid groups are linked with two carbon atoms which form part of a hydrocarbon radical that may or may not be substituted and which has 2 to 8 carbon atoms, which acid has electrolytic dissociation constants smaller than  $2.3 \times 10^{-4}$ , the said light-sensitive layer containing a quantity of said acid equimolarly corresponding to at least 0.20 g. of succinic acid per m.<sup>2</sup> of its light-sensitive surface. Semi-wet development of said diazotype material with the usual developers reacting moderately alkaline yields azo-dyestuffs with attractive pure (and neutral) shades of colour. Fluctuations in the application or concentration of the developer have a much smaller influence on the shade of the azo-dyestuffs when diazotype material according to the invention is used than if use is made of similar diazotype materials containing the usual acids, such as citric acid and tartaric acid. Upon ageing, diazotype material according to the invention further shows less loss of its mechanical strength. By the use of one-component diazotype material according to the invention it is possible to achieve, with one and the same developer reacting moderately alkaline, a substantially complete development—which is only slightly affected, if at all, by development fluctuations—both of transparent diazotype material sensitized with actively coupling diazo compounds which upon semi-wet development give azo-dyestuffs with a high absorption for ultra-violet light, such as p-diazo o-chloro N,N-diethylaniline, and of diazotype material sensitized with very actively coupling diazo compounds, such as 4-diazo 2,5-dialkoxy acylanilides, 4-diazo 2,5-dialkoxy arylmercaptobenzene compounds, and 4-diazo 2,5-dialkoxy diphenyl compounds.

With the azo coupling components normally used in the semi-wet diazotype process, for example, with phloroglucinol and resorcinol, the very actively coupling compounds of the said groups yield azo-dyestuffs which are highly resistant to oxidation and to the action of light. Moreover, the photo-decomposition products which remain in the exposed portions of the diazotype copy after the imagewise exposure of the diazotype material sensitized with these very actively coupling diazo compounds are highly resistant to oxidation or to the action of light. The azo-dyestuffs of the said very actively coupling diazo compounds do not, however, have high absorption for ultra-violet light, so that these diazo compounds are not particularly suited for the sensitization of transparent diazotype materials which are used for the production of intermediate copies. However, there are other actively coupling compounds, such as p-diazo o-chloro N,N-diethylaniline and p-diazo o-methyl N,N-diethylaniline, which with phloroglucinol and resorcinol yield azo-dyestuffs which possess very high absorption for ultra-violet light and which are therefore very suitable for the manufacture of transparent diazotype material. Such transparent material is not suited for semi-wet development with weakly alkaline to weakly acidic buffered developers, because during development the pH of the surface of the diazotype material is still too low in relation to the coupling activity of the diazo compound, though this activity

is large. The diazo compound is not completely converted into azo-dyestuff. This is called "underdevelopment." Said transparent diazotype materials are, however, well suited for semi-wet development with the said developers reacting moderately alkaline.

In practice transparent and non-transparent diazotype materials are preferably developed with one and the same developer.

The acids included in the diazotype material according to the invention are in general readily available. Those with a relatively low molecular weight are sufficiently soluble in aqueous liquids which are used for the manufacture of one-component diazotype material, for example, sensitizing liquids or pre-coating liquids. Those with a relatively high molecular weight dissolve sufficiently in liquids containing a sufficient quantity of an organic solvent, such as methyl alcohol, ethyl alcohol, acetone, and the like. The differences between the two dissociation constants of the said aliphatic saturated dicarboxylic acids are considerably smaller than those present in other organic di- or tricarboxylic acids, such as oxalic acid, tartaric acid, citric acid or maleic acid. The last-mentioned acids have a first electrolytic dissociation constant which is considerably greater than  $2.3 \times 10^{-4}$ . The hydrocarbon radical with which the two carboxylic acid groups in the acids applied in the diazotype material according to the invention, are linked may or may not be branched; it is also possible for one or more hydrogen atoms of the hydrocarbon radical to be replaced by groups other than carboxylic acid groups, for example, by amino-, mono-, and dialkylamino groups; the carboxylic acid groups may be linked with two adjacent carbon atoms or with two carbon atoms which are further apart. Suitable acids are, for example, succinic acid, glutaric acid, adipic acid, pimelic acid, suberic acid, azelaic acid, sebacic acid, anti-dimethyl succinic acid, ethyl-succinic acid,  $\beta, \beta$ -dimethyl glutaric acid,  $\beta$ -methyl adipic acid, aspartic acid and glutamic acid.

The acid content of the light-sensitive layer of one-component diazotype material according to the invention may vary according to the variation of the diazo content.

In order to avoid the objectionable consequences of development fluctuations, however, a relatively high acid content of the light-sensitive layer of the one-component diazotype material is always needed.

The acid content may be relatively larger as the coupling activity of the diazo compounds used is greater. In order to achieve substantially complete development of one-component diazotype material containing only the usual acids, such as citric acid and tartaric acid, a precise quantity of these acids is necessary when a given developer reacting moderately alkaline is used. A small excess of the acids causes under-development, a small shortage of the acids causes over-development. The acid content of the one-component diazotype material according to the invention may vary within much wider limits without causing over- or under-development.

For the manufacture of one-component diazotype material according to the invention it is not necessary to replace the quantity of citric acid or other conventional acid in a given one-component diazotype material by an equivalent quantity of acid according to the invention. It is possible to use considerably more than the equivalent quantity of the last-mentioned acid. The larger the quantity of this acid that can be applied, the better can the detrimental consequences of development fluctuations be avoided, while the drawbacks involved in a high acid content of the light-sensitive layer do not appear or, in a much lower degree, than if use is made of a similar diazotype material with a high content of a conventional acid, such as citric acid or tartaric acid.

As appears from the above description, there are differences in coupling activity between the actively coupling diazo compounds suitable for application in one-component diazotype material according to the invention.

The avoidance of the detrimental consequences of de-

velopment fluctuations in general is greatest upon the use of diazo compounds with the greatest coupling activity. Very good results are obtained with one-component diazotype material according to the invention in which the actively coupling diazo compound is a compound of the type:

10



in which X is an anion and R an alkyl or aralkyl group. The acyl group may be, for example, acetyl, propionyl, benzoyl, p-chloro-benzoyl, phenyl-acetyl or phenoxyacetyl. A familiar compound of this type is, for example, the 4-benzoylaminobenzene diazonium chloride, zinc chloride double salt.

Good results are also obtained with one-component diazotype material according to the invention in which the actively coupling diazo compound is a compound of the type:

25



in which X is an anion, R an alkyl or aralkyl group, and R1 an aryl group that may or may not be substituted. A suitable compound of this type is, for example, the 2,5-dimethoxy-4-(p-tolylmercapto)-benzene diazonium chloride, zinc chloride double salt. See also German Patent No. 896,591 and British specification No. 759,045.

35 In another favourable one-component diazotype material according to the invention the actively coupling diazo compound is a compound of the type

40



in which X is an anion, R an alkyl or aralkyl group, and R1 an aryl group that may or may not be substituted. A suitable compound of this type is, for example, 1-diazo 2,5-dimethoxy-4'-methoxydiphenyl.

45 The formation of black azo-dyestuffs by the semi-wet development of one-component diazotype material according to the invention with a developing liquid reacting moderately alkaline and containing phloroglucinol can be promoted by using in the developing liquid, or in the light-sensitive layer of the diazotype material, a compound which is able to form an addition compound with phloroglucinol, such as antipyrine and pyramidon, or xanthines, such as caffeine, theobromine or theophylline.

50 Attractive black azo-dyestuff images can thus be obtained with one-component diazotype material according to the invention the light-sensitive layer of which contains a xanthine.

55 The diazotype material according to the invention may contain the auxiliary substances commonly used in one-component diazotype materials, for example, means preventing the discoloration of diazotype copies, such as thiourea, constituents facilitating the sensitization, such as gelatin, gum arabic and isopropyl alcohol; substances which prevent curling, such as glycerol and polyethylene glycol; means promoting the uniformity of the light-sensitive layer, such as dispersions of silica, aluminium oxide, titanium dioxide, barium sulphate, synthetic resins and unboiled starches such as rice starch; means preventing ink-feathering in writing or drawing on copies on such material, such as water-soluble salts of sym. diaryl-

guanidines, for example, sym. diphenylguanidine; stabilizers, for example, acids or acid salts such as citric acid, tartaric acid, alum and 1,3,6-naphthalene trisulphonic acid. However, no large quantities of the said acids or acid salts must be used, since otherwise no substantially complete development will be achieved with developers reacting moderately alkaline.

An excellent keeping quality is shown by one-component diazotype material according to the invention the light-sensitive layer of which contains a mixture of boric acid and an organic hydroxy acid capable of forming a complex with boric acid. A small quantity of a mixture of boric acid and tartaric acid or boric acid and citric acid is sufficient.

The following examples will serve to illustrate the invention:

*Example I*

White base-paper for the diazotype process of weight 80 g./m.<sup>2</sup> is sensitized with a solution of:

20 g. of p-4'-methyl phenylmercapto-2,5-dimethoxybenzene diazonium chloride, zinc chloride double salt  
50 g. of succinic acid  
2 g. of thiourea  
35 g. of rice starch  
30 cm.<sup>3</sup> of a dispersion of polyvinylacetate (Vinnapas H.60)  
1000 cm.<sup>3</sup> of water

and dried.

The sensitized surface contains approximately 0.2 g. of the diazo compound and approximately 0.5 g. of succinic acid per m.<sup>2</sup>. Under a transparent original drawn in pencil a sheet of the diazotype paper is exposed in an exposure apparatus equipped with a high-pressure mercury vapour lamp until the portions of the light-sensitive layer lying under the transparent portions of the original are substantially (not completely) bleached, as is customary in practice when making copies of pencil-drawings. The imagewise exposed sheet is developed by applying approximately 8 g./m.<sup>2</sup> of the following developing liquid:

30 g. of thiourea  
6.5 g. of phloroglucinol  
6.5 g. of resorcinol  
1 g. of potassium salt of hydroquinone mono-sulphonic acid  
1.5 g. of sodium salt of dibutylnaphthalene sulphonic acid commercially available under the name Sorbit P (in the following examples briefly referred to as Sorbit P)  
25 g. of mannitol  
80 g. of potassium tetraborate pentahydrate  
10 g. of potassium carbonate  
1000 cm.<sup>3</sup> of water

This developing liquid has a pH of 9.4.

The developed copy shows a strong black positive image on a foggy background. If the concentration of the constituents of this developer has increased, for example, in consequence of evaporation of the developer in the developing apparatus, to such an extent that the original volume of 1050 cm.<sup>3</sup> has decreased to about 700 cm.<sup>3</sup>, upon development of a copy on this light-sensitive material in an otherwise similar way an image is obtained of which the shade of the azo-dyestuff does not deviate substantially from that of the image obtained with the normally concentrated developer.

If, instead of 50 g. of succinic acid, 40 g. of citric acid or 45 g. of tartaric acid or 30 g. of maleic acid is used in the sensitizing liquid, a substantially complete development is indeed obtained with the above-mentioned normally concentrated developer, but with the developer evaporated to 700 cm.<sup>3</sup> a brown-violet instead of a black azo-dyestuff shade is obtained.

*Example II*

White base-paper for the diazotype process of weight 80 g./m.<sup>2</sup> is sensitized with a solution of:

5 20 g. of p-4'-methoxy phenyl 2,5-diethoxybenzene diazonium chloride, zinc chloride double salt  
45 g. of glutaric acid  
1 g. of gelatin in  
1000 cm.<sup>3</sup> of water

10 and dried.

The sensitized surface contains approximately 0.21 g. of the diazo compound and approximately 0.45 g. of glutaric acid per m.<sup>2</sup>.

A sheet of the diazotype paper is imagewise exposed as described in Example I.

The imagewise exposed sheet is developed by applying approximately 8 g./m.<sup>2</sup> of the following developing liquid:

26 g. of thiourea  
6.5 g. of phloroglucinol  
20 6.5 g. of resorcinol  
1.5 g. of Sorbit P  
3 g. of sodium salt of ethylene diamine tetra-acetic acid  
32 g. of sodium carbonate  
1000 cm.<sup>3</sup> of water

25 This developing liquid has a pH of 9.5.

The developed copy shows a strong black positive image on a foggy background with little variation of shade in consequence of development fluctuations. If, instead of 45 g. of glutaric acid, 33 g. of ortho-phosphoric acid or 50 g. of alum or 40 g. of aluminium sulphate is used in the sensitizing liquid, considerable variations in azo-dyestuff shade owing to development fluctuations are obtained.

*Example III*

White base-paper for the diazotype process of weight 80 g./m.<sup>2</sup> is sensitized with a solution of:

30 30 g. of p-benzoylamido-2,5-di-n-propoxy benzene diazonium chloride, zinc chloride double salt  
40 70 g. of  $\beta$ -methyl adipic acid  
20 g. of caffeine  
2.5 g. of gelatin in  
1000 cm.<sup>3</sup> of water

and dried.

45 The sensitized surface contains approximately 0.25 g. of the diazo compound and approximately 0.58 g. of  $\beta$ -methyl adipic acid per m.<sup>2</sup>. A sheet of the diazotype paper is exposed and developed as described in Example I.

50 The developed copy shows a strong black positive image on a foggy background with little variation of shade in consequence of development fluctuations.

*Example IV*

Paper of weight 150 g./m.<sup>2</sup>, one side of which has been 55 coated with a cellulose acetate layer (approximately 50% by weight of combined acetic acid) with a thickness of about 10 microns, which has been fixed to the paper by means of an adhesive and which has been deacylated to a depth of about 4 microns and to an average acetyl content, calculated as combined acetic acid, of approximately 20% by weight (which corresponds to an average number of acyl groups linked with the OH-groups of 0.7), is 60 impregnated on the deacylated side of the cellulose acetate layer during 30 seconds with the following solution:

65 65 g. of p-4'-methyl phenylmercapto 2,5-diethoxy benzene diazonium chloride, zinc chloride double salt  
2 g. of alum

300 cm.<sup>3</sup> of ethyl alcohol (96%) in  
700 cm.<sup>3</sup> of water

70 dried, treated further with a solution of:

75 75 g. of suberic acid in  
1000 cm.<sup>3</sup> of ethyl alcohol (96%)

75 and dried again.

Before drying, the excess of liquid is removed each time from the cellulose acetate surface. The sensitized surface contains approximately 0.28 g. of the diazo compound and approximately 0.9 g. of suberic acid per m.<sup>2</sup>. A sheet of the diazotype paper is exposed under a transparent original drawn in ink until the portions of the light-sensitive layer lying under the transparent portions of the original are completely bleached out. The imagewise exposed sheet is developed by applying approximately 9 g./m.<sup>2</sup> of the following developing liquid:

30 g. of thiourea  
6.5 g. of phloroglucinol  
6.5 g. of resorcinol  
1 g. of potassium salt of hydroquinone mono-sulphonic acid  
1.5 g. of Sorbit P  
5 g. of sorbitol  
15 g. of beet sugar  
55 g. of potassium tetraborate pentahydrate  
12 g. of potassium hydroxide  
1000 cm.<sup>3</sup> of water

The developing liquid has a pH of 9.4.

The developed copy shows a strong black positive image on a bright white background with few deviations in shade, if any, in consequence of vibrations and mechanical irregularities of the developing apparatus.

If the light-sensitive surface contains 0.42 g. of citric acid instead of 0.9 g. of suberic acid, considerable differences in azo-dyestuff shades are obtained in consequence of vibrations and mechanical irregularities of the developing apparatus, for example, in the form of alternating green-black, black, and brown-black streaks in the azo-dyestuff image.

#### Example V

White base-paper for the diazotype process of weight 80 g./m.<sup>2</sup> is pre-coated with approximately 15 g./m.<sup>2</sup> of an aqueous polymeric methacrylic acid ester dispersion diluted with water in a proportion of 1 part to 5 parts of water, in which 0.1% by weight of Tylose SL 25 has been dissolved.

It is dried in a current of air at 100° C. The surface thus treated is sensitized with a solution of:

15 g. of p-4'-methyl phenyl-mercaptop-2,5-diethoxy-benzene diazonium chloride, zinc chloride double salt  
5 g. of p-benzoylamido 2,5-diethoxy benzene diazonium chloride, zinc chloride double salt  
40 g. of succinic acid  
12 g. of adipic acid  
2 g. of boric acid  
5 g. of tartaric acid  
2 g. of thiourea  
10 g. of caffeine  
2.5 g. of gelatin in  
1000 cm.<sup>3</sup> of water

and dried.

The sensitized surface contains about 0.15 g. of the mercapto-diazo compound, about 0.05 g. of the acylamido diazo compound, about 0.4 g. of succinic acid and about 0.12 g. of adipic acid per m.<sup>2</sup>.

A sheet of the diazotype paper is exposed and developed as described in Example I.

The developed copy shows a strong black image on a foggy background with little variation of shade in consequence of development fluctuations.

#### Example VI

White base-paper for the diazotype process of weight 80 g./m.<sup>2</sup> is sensitized with a solution of:

23 g. of p-4'-methyl phenylmercaptop-2,5-diethoxy benzene diazonium chloride, zinc chloride double salt  
20 g. of caffeine  
30 g. of succinic acid

20 cm.<sup>3</sup> of a dispersion of polyvinyl acetate (Rhodopa 6000) in  
1000 cm.<sup>3</sup> of water

and dried.

The sensitized surface contains approximately 0.2 g. of the diazo compound and approximately 0.26 g. of succinic acid per m.<sup>2</sup>. A sheet of the diazotype paper is imagewise exposed as described in Example I.

The imagewise exposed sheet is developed by applying approximately 8 g./m.<sup>2</sup> of the following developing liquid:

6.5 g. of phloroglucinol  
6.5 g. of resorcinol  
1 g. of potassium salt of hydroquinone monosulphonic acid  
1.5 g. of Sorbit P  
10 g. of beet sugar  
70 g. of potassium tetraborate pentahydrate  
20 g. of benzoic acid  
1000 cm.<sup>3</sup> of water

The developing liquid has a pH of 8.4.

The developed copy shows a strong black image on a foggy background with little variation of shade in consequence of development fluctuations.

What we claim is:

1. A one-component diazotype material comprising paper having a fibrous side thereof sensitized by a light-sensitive composition containing, and in the absence of an azo coupling component, an actively coupling light-sensitive diazo compound of the formula



40 in which X is an anion, R is a radical selected from the group consisting of alkyl and aralkyl radicals, and Y is a radical selected from the group consisting of acylamino, arylmercapto, and aryl radicals, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side.

45 2. A one-component diazotype material comprising paper having a fibrous side thereof sensitized by a light-sensitive composition containing, and in the absence of an azo coupling component, an actively coupling light-sensitive diazo compound of the formula



50 in which X is an anion and R is a radical selected from the group consisting of alkyl and aralkyl radicals, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side.

55 3. A one-component diazotype material comprising paper having a fibrous side thereof sensitized by a light-sensitive composition containing, and in the absence of

an azo coupling component, an actively coupling light-sensitive diazo compound of the formula



in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side.

4. A one-component diazotype material comprising paper having a fibrous side thereof sensitized by a light-sensitive composition containing, and in the absence of an azo coupling component, an actively coupling light-sensitive diazo compound of the formula



in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side.

5. A one-component diazotype material comprising paper having a fibrous side thereof sensitized by a light-sensitive composition containing, and in the absence of an azo coupling component, an actively coupling light-sensitive diazo compound of the formula



in which X is an anion, R is a radical selected from the group consisting of alkyl and aralkyl radicals, and Y is a radical selected from the group consisting of acylamino, arylmercapto, and aryl radicals, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing a xanthine.

6. A one-component diazotype material comprising paper having a fibrous side thereof sensitized by a light-sensitive composition containing, and in the absence of an azo coupling component, an actively coupling light-sensitive diazo compound of the formula



in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing a xanthine.

yllic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing a xanthine.

7. A one-component diazotype material comprising paper having a fibrous side thereof sensitized by a light-sensitive composition containing, and in the absence of an azo coupling component, an actively coupling light-sensitive diazo compound of the formula



in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing a xanthine.

8. A one-component diazotype material comprising paper having a fibrous side thereof sensitized by a light-sensitive composition containing, and in the absence of an azo coupling component, an actively coupling light-sensitive diazo compound of the formula



40 in which X is an anion, R is a radical selected from the group consisting of alkyl and aralkyl radicals, and Y is a radical selected from the group consisting of acylamino, arylmercapto, and aryl radicals, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing boric acid and an organic hydroxy compound capable of forming a complex with boric acid.

45 9. A one-component diazotype material comprising paper having a fibrous side thereof sensitized by a light-sensitive composition containing, and in the absence of an azo coupling component, an actively coupling light-sensitive diazo compound of the formula



in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing boric acid and an organic hydroxy compound capable of forming a complex with boric acid.

13

10. A one-component diazotype material comprising paper having a fibrous side thereof sensitized by a light-sensitive composition containing, and in the absence of an azo coupling component, an actively coupling light-sensitive diazo compound of the formula



in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing boric acid and an organic hydroxy compound capable of forming a complex with boric acid.

11. A one-component diazoty material comprising paper having a fibrous side thereof sensitized by a light-sensitive composition containing, and in the absence of an azo coupling component, an actively coupling light-sensitive diazo compound of the formula



in which X is an anion, R is a radical selected from the group consisting of alkyl and aralkyl radicals, and Y is a radical selected from the group consisting of acylamino, arylmercapto, and aryl radicals, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing a xanthine and boric acid and an organic hydroxy compound capable of forming a complex with boric acid.

12. A one-component diazotype material comprising paper having a fibrous side thereof sensitized by a light-sensitive composition containing, and in the absence of

14

an azo coupling component, an actively coupling light-sensitive diazo compound of the formula



10 in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants 15 of said acid being smaller than  $2.3 \times 10^{-4}$ , said composition providing at least 1.7 millimols of said acid per square meter of the area of said side, said composition also containing a xanthine and boric acid and 20 an organic hydroxy compound capable of forming a complex with boric acid.

plex with boric acid.

13. A one-component diazotype material comprising paper having a fibrous side thereof sensitized by a light-sensitive composition, containing, and in the absence of an azo coupling component, an actively coupling light-sensitive diazo compound of the formula



in which X is an anion, R is a radical selected from the group consisting of alkyl and aralkyl radicals and R<sub>1</sub> is an aryl radical, and containing with said compound an aliphatic saturated dicarboxylic acid in which the carboxylic acid radicals are linked with two carbon atoms forming part of a hydrocarbon radical having from 2 to 8 carbon atoms, the electrolytic dissociation constants of said acid being smaller than  $2.3 \times 10^{-4}$ , said composition providing at least 1.7 millimols of said acid per square meter of the area of said side, said composition also containing a xanthine and boric acid and an organic hydroxy compound capable of forming a complex with boric acid.

**References Cited in the file of this patent**

UNITED STATES PATENTS

- 1,870,930 Spongerts ----- Aug. 9, 1932  
2,405,523 Sease et al. ----- Aug. 6, 1946

## FOREIGN PATENTS

- 415.081 Great Britain ----- Aug. 16, 1934